

C. T. TORSSELL,  
MANUFACTURE OF COMBINED STEEL INGOTS AND PLATES.  
APPLICATION FILED MAY 25, 1910.  
987,774. Patented Mar. 28, 1911.  
2 SHEETS—SHEET 1.



Witnesses.

L. A. Williams  
W. A. Knittle

Inventor:  
Carl T. Torsell  
by John H. Roney  
his Attorney.

C. T. TORSSELL.

MANUFACTURE OF COMBINED STEEL INGOTS AND PLATES.

APPLICATION FILED MAY 25, 1910.

987,774.

Patented Mar. 28, 1911.

2 SHEETS—SHEET 2.



*Fig. 6.*

*Fig. 7.*



*Witnesses,*

*C. A. Williams*  
*E. N. Hicks*

*Inventor:*  
*Carl T. Torsell*

*by John H. Roney*  
*Attorney.*

# UNITED STATES PATENT OFFICE.

CARL T. TORSELL, OF WARREN, OHIO.

## MANUFACTURE OF COMBINED STEEL INGOTS AND PLATES.

987,774.

Specification of Letters Patent. Patented Mar. 28, 1911.

Application filed May 25, 1910. Serial No. 563,246.

To all whom it may concern:

Be it known that I, CARL T. TORSELL, a subject of the King of Sweden, residing at Warren, in the county of Trumbull and State of Ohio, have invented a new and useful Improvement in the Manufacture of Combined Steel Ingots and Plates, of which improvement the following is a specification.

My invention relates to the manufacture of what are known as combined steel plates, viz., steel plates having layers of different hardness due to the different carbon content thereof, or other elements, as for instance, a layer of high carbon or hard steel on the outer side and a central layer of low carbon or soft steel or iron, so as to render the composite plate not only hard but also tough. In the manufacture of this type of plate where the hard steel entirely surrounds the soft, as in the usual practice, it is impossible to prevent or avoid the making of very considerable waste, frequently from ten to fifteen per cent. of the entire plate, due to the fact that the hard steel overlaps the soft and after rolling necessitates the cutting off the sides of the plates in order to expose the soft central layer thereof.

The principal object of this present invention is to prevent this waste, or at least to reduce it to a possible minimum, and I accomplish this object by the following method of manufacture.

In the practice of my invention I preferably form an ingot as follows: I place the central soft layer in a mold of suitable construction in such position in said mold that the hard molten metal when poured therearound completely surrounds the same, excepting at that part of the ingot where a portion of the soft central layer is exposed at both sides, as illustrated in Fig. 1 of the accompanying drawings. I also preferably in the practice of my invention proportion the exposed portion of the soft central portion of the ingot relative to the unexposed portion thereof. While I do not limit or confine myself to the exact proportions, good efficiency can be obtained by making the exposed portion of the soft central portion of the ingot about one-third the thickness thereof, and about equal to each of the engaging portions of the outer layers or hard portions of the ingot as will be noticed in said figure.

In the accompanying drawings I have

shown my invention in its various stages, first as an ingot and subsequently reduced to a plate, and the rolls employed in performing the operation.

In said drawings Figure 1 is a transverse section of the ingot. Fig. 2 is a view of the plate, partly in section; and, Fig. 3 is a sectional view of the ingot being subject to one pass of the roll; Fig. 4 is a similar view, the ingot being turned edgewise with relation to its component layers; Fig. 5 is a transverse section of a five layer ingot suitable for the production of safe plates, etc. Fig. 6 is a perspective view of the ingot when formed. Fig. 7 is a side elevation of the same.

Referring to the drawings, 1, 2, are outer layers of hard steel; 3 is a central soft layer, the said layer 3 having grooves 4, and projections 5, along the sides thereof, in which the hook-like portions 6, 7, of the layers 1 and 2 engage, it being understood that the said outer layers are poured around the central layer and that the molten metal flows into the recesses specified and over the projections constituting an integral ingot, composed of three layers. The hook portions of the outer layers and recesses of the central layer forming mechanical means for securing the layers together.

Another essential feature of the invention is that the exposed portions 8, of the central layer should project out on a line with the outer edge of the two remaining layers which surrounds it. It is also understood that the ingot when cast is subsequently heated and brought to a suitable temperature to enable the same to be thoroughly welded or reduced either by rolls or other compression.

In the drawings I have shown that the ingot when heated is passed through the rolls 9, 9, sidewise and the edgewise portion of the roll on the second pass. I have merely mentioned these passes as illustrative, as it is manifest that one or more passes sidewise may be made before any edgewise pass is performed, or vice versa.

I have not shown a mold in connection with the production of my improved ingot, as any suitable mold may be employed in which the central soft layer can be supported above the bottom of the mold in such wise as to permit the molten hard metal to be poured completely around the same as shown in Fig. 1. Nor have I shown any

heating furnace, as any suitable furnace for heating the ingot may be employed.

I have demonstrated by practice that the ingot produced as described can be rolled down to a plate 10, or slab, with a minimum of waste along the sides, and a uniformity of reduction in the layers thereof, so as to produce a plate having three distinct layers of substantially uniform thickness through the entire width, and completely and thoroughly welded together.

Having described my invention, what I claim and desire to secure by Letters-Patent is:

15 1. The herein described method of casting an ingot formed of several layers, which consists in forming recesses along the edges of the intermediate layers and casting the molten metal constituting the outer or surrounding portion of the ingot therearound, with the mid portion of the edges of the intermediate layers exposed, and with the top and bottom thereof completely surrounded, whereby the said layers are so 20 united that the admission of air is prevented between the surfaces of said layers.

25 2. The herein described method of casting an ingot, comprising several layers, which consists in forming recesses along the entire

edges of the central layer and casting the 30 molten metal constituting the outer or surrounding portion of the ingot around said central layer, the molten metal flowing into said recesses and completely over the top and bottom of the central layer, whereby the 35 several layers constituting the ingot are so united that the admission of air between the surfaces of the said layers is prevented.

3. A combined steel ingot having the central portion of the side of the central layer 40 exposed, and the outer layers overlapping the edges of the central layer and completely surrounding the top and bottom of said central layer.

4. A combined steel ingot comprising several layers, the intermediate layer having the central portion of the sides thereof exposed, and the top and bottom thereof completely surrounded by the overlapping outer 45 layers. 50

In testimony whereof, I have hereunto signed my name in the presence of two subscribing witnesses.

CARL T. TORSSELL.

In the presence of—

JOHN H. RONEY,

CLARENCE A. WILLIAMS.